

27

Aug. 1, 1933.

Metallic

4

Search Room

D. FINLEY

1,920,931

ROOFING MATERIAL

Filed Feb. 17, 1930

T1849

X1853

X1962

X1909

X148/228



INVENTOR  
 DOZIER FINLEY  
 BY *Charles S. Evans*  
 HIS ATTORNEY.

4

Patented Aug. 1, 1933

1,920,931

## UNITED STATES PATENT OFFICE

1,920,931

## ROOFING MATERIAL

Dozier Finley, Berkeley, Calif., assignor to The Paraffine Companies, Inc., San Francisco, Calif., a Corporation of Delaware

Application February 17, 1930. Serial No. 429,040

3 Claims. (Cl. 91—68)

My invention relates to roofing material and particularly to such material having a metallic coating.

One of the objects of the invention is the provision of a roofing material in which the metallic coating can not be stripped off the body of the material, and hence is subject to minimum damage from handling.

Another object of the invention is the provision of a metallic coated roofing which is flexible and of light weight.

A further object of the invention is the provision of a metallic coated roofing in which a wide variety of metallic substances may be used, and hence, a wide range of colors and textures made possible.

The invention possesses numerous other objects and features of advantage, some of which, with the foregoing, will be set forth in the following description of my invention. It is to be understood that I do not limit myself to this disclosure of species of my invention, as I may adopt variant embodiments thereof within the scope of the claims.

The figure of the drawing is a perspective view of a piece of roofing embodying the invention.

In the practice of making metal clad roofing materials, it has been customary to apply the metal coating over a granular mineral surfaced composition base, by an electroplating process. This roofing involves considerable expense in manufacture, is restricted to the choice of metals used, and is no lighter in weight than the usual granule surfaced roofing, since it contains granules plus the additional metal coating.

When an electroplated roofing is laid in shingle form it suffers in appearance from loss in shadow lines, because the edges are covered with metal and consequently do not give a contrasting color with relation to the top surface of the shingle.

Furthermore, when a composition base is covered with a sheet of metal there is grave danger of the metal becoming loosened or even stripped from the surface during shipment or other handling. Once removed, the metal coating is difficult to replace in original form.

This invention overcomes the above mentioned difficulties; and at the same time embodies those other features of appearance and protection which are desirable in roofing materials.

In terms of broad inclusion the invention comprises a body layer of decay-resistant material impervious to moisture, and having a covering of metallic granules fixed thereon. Preferably a

base of treated fibrous material is provided underlying the body. The roofing material may be formed in sheets or shingles, depending on the mode of application.

In greater detail the invention comprises a body layer or coating 2 of decay-resistant mastic material which is impervious to moisture. A bituminous compound such as coal tar or asphalt possesses these qualities, and such a compound of medium hard grade is preferably used for this purpose.

In order to give sufficient rigidity to the roofing material a base layer 3 is preferably provided underlying the body layer or coating 2. The base 3 is preferably of fibrous material such as the felt ordinarily used in the manufacture of felt base roofing; and is preferably treated with a bituminous saturant in the manner well known to those skilled in the art of making felt base roofing.

The body layer 2 is formed as a coating on the upper side of the base 3 and is applied in fluid state according to well known practice. A thin coating layer 4, preferably of a bituminous compound similar to that used for the body layer, is preferably formed on the lower side of the base 3 to give added protection thereto.

A covering layer 6 of metallic granules, overlying the body layer or coating 2, is preferably applied while the mastic layer is in a soft state. The whole is then preferably rolled to evenly embed the granules in the surface of the body layer. The granules 6 may be of any metallic substance such as bits of sheet metal, fine shot or filings.

A particular feature of advantage of the invention resides in the fact that the granules 6 are secured to the roofing material by embedding them in a mastic layer. This permits the use of any kind or shape of metallic granules that may be desired. One type of granule that has proven very effective is made by cutting up into small pieces, thin sheets of pure metal, such as rolled copper plate, thus producing flat angular particles of the metal. Also, granules in the nature of filings, made by a cutting tool such as a file or a rotary tool of the milling cutter type, give striking results when used in accordance with the terms of the invention. Fine metallic shot, the making of which is a well known process, is another of the many forms which the granules 6 may take; and these may be used in original form or they may first be flattened.

Surfacing roofing materials with metallic granules as herein disclosed, permit the use of me-

tallic granules other than the usually more expensive pure metals. It is possible to use granules composed of a cheap base metal, or mineral, plated with a more expensive metal. Also, 5 bimetallic granules may be used, and striking color variations can be secured in this manner. These granules may easily be made from a bimetallic plate comprising a sheet of inexpensive metal on which a coating, such as copper, has 10 been plated; the composite sheet being cut into small angular particles as previously described, either before or after plating.

It is also possible to use alloys for making 15 the granules, and very good effects are produced by using brass or bronze in this manner. Still another of the many possibilities in making the granules is to plate galvanically a pure metal, or a composite sheet of different metals, on a travelling belt, and then strip the deposit from 20 the belt and cut it up into small angular particles. In fact, the use of metallic granules in this manner offers almost an endless number of possibilities, because their application on the roofing material does not depend on any particular 25 characteristic of the metal or metallic particles used.

While it might be thought that the non-corrodible metallic particles are to be preferred to those easily and quickly corroded, yet the invention 30 is not confined to metals difficult to corrode or corrosion-proof metals. For instance iron particles may be used. It is found that the iron granules will give the harmonizing color effects of a soft brownish or reddish brown color with 35 traces of almost black when corroded.

Ordinary corrosion of iron particles on a roof will produce a hard scale-like product of corro-

sion many times larger in bulk than the original iron particles, and while some may be lost, a sufficient amount will stay in place to serve as an ideal covering for the asphaltic layer below. In fact, the corrosion product, being several times the volume of the parent material, will tend to seal over all parts of the cementing asphalt, inclusive particularly of the many tiny areas not originally covered by the metallic particles. A minor amount of the ferrous corrosion may be had by using some of the more slowly corrodible forms of iron or steel, such as copper bearing steel, the "stainless steels" or similar alloys.

The roofing material may either be formed in sheets or in shingles, depending upon the method of application to a roof. If the material is to be used in sheet form, its flexibility permits it to be readily rolled up in convenient form for distribution and sale.

I claim:

1. A roofing material comprising a moisture-proof layer, and a variegated surface layer of bimetallic granules, said granules being of one metal partially coated with a metal of different color.

2. A roofing material comprising a bituminous layer, and a variegated covering layer of substantially flat angular bi-metallic granules overlying and partially embedded in the bituminous layer.

3. A roofing material comprising a bituminous layer and a variegated surface covering layer of bi-metallic granules partially embedded in the bituminous layer, said granules being in the form of particles cut from metallic plates each plate being coated on one side with a different metal.

40

115

45

120

50

125

55

130

60

135

65

140

70

145

75

150

80

85

90

95

100

105

110

DOZIER FINLEY.